

# UNITED STATES PATENT OFFICE.

WALTER E. WRIGHT, OF CLEVELAND, OHIO.

## PAINT.

1,308,884.

Specification of Letters Patent.

Patented July 8, 1919.

No Drawing.

Application filed August 3, 1917. Serial No. 184,207.

To all whom it may concern:

Be it known that I, WALTER E. WRIGHT, a citizen of the United States, residing at Cleveland, in the county of Cuyahoga and 5 State of Ohio, have invented a new and useful Paint, of which the following is a specification.

This invention relates to an improved paint more especially adapted for an under- 10 coat in painting and comprising a suitable metallic pigment, tung oil, a semi-drying or non-drying oil adapted to retard the drying of the tung oil, a drying oil other than tung oil, as, for instance, linseed oil, and a thinning vehicle, such, for instance, as turpen- 15 tine or petroleum distillate.

The object of this invention is to produce a paint which is not only more especially adapted for an undercoat in painting, but 20 which insures a slow-drying undercoat and produces a better surface to receive the finishing coat of paint and is more alkali- 25 resisting, more easily applied and more durable than undercoats of paints heretofore used.

The present invention more especially pertains to a paint comprising a suitable metallic pigment, such, for instance, as white lead or oxid of zinc. A lead pigment is prefer- 30 ably used in making my improved paint which also comprises the strongest drying vegetable oil known, viz., tung oil. Tung oil is an indispensable drying oil in the production of my improved paint which also 35 comprises a semi-drying oil, such, for instance, as soja bean oil or cotton-seed oil, or a non-drying oil, such, for instance, as paraffin oil. My improved paint also comprises a suitable drying oil other than tung 40 oil, as, for instance, linseed oil, and linseed oil is preferred because it dries with a tough and elastic skin and is therefore a most de- 45 sirable oil as a binder in making my im- proved paint. I would here remark that the drying of the linseed oil and tung oil, and more especially the drying of the tung oil, is retarded by the use of soja bean oil or cotton-seed oil or paraffin oil. The use of soja bean oil in retarding the drying of the 50 tung oil is preferred, but I would here re- mark that soja bean oil of itself dries tacky and would be undesirable and impractical without the presence of a suitable quantity of tung oil. Of course, my improved paint 55 also comprises a suitable thinning vehicle,

such, for instance, as turpentine or petroleum distillate.

In making my improved paint I prefer- 60 ably use the metallic pigment, the tung oil, the oil adapted to retard the drying of the tung oil, linseed oil as the drying oil other than tung oil, and the thinning vehicle sub- 65 stantially in the proportion, by weight, of from four to fourteen parts of the tung oil, from seven to thirty-five parts of the oil 70 adapted to retard the drying of the tung oil, from nine to twelve parts of the linseed oil, and from eighteen to twenty-four parts of the thinning vehicle, to one hundred parts of the pigment.

Good results have been attained by me in 75 using a lead or zinc pigment, linseed oil, tung oil, soja bean oil and a thinning vehicle, substantially in the proportion, by weight, of from nine to twelve parts of lin- 80 seed oil, eight parts of tung oil, twenty parts of soja bean oil and from eighteen to twenty-four parts of the thinning vehicle to one hundred parts of the pigment.

Good results have been attained by me in 85 using a lead or zinc pigment, linseed oil, tung oil, soja bean oil and a thinning vehicle substantially in the proportion, by weight, of from nine to twelve parts of linseed oil, fourteen parts of tung oil, thirty-five parts 90 of soja bean oil and from eighteen to twenty-four parts of the thinning vehicle to one hundred parts of the pigment.

Fairly good results have been attained by 95 me in using a lead or zinc pigment, linseed oil, soja bean oil and a thinning vehicle sub- 100 stantially in the proportion, by weight, of from nine to twelve parts of linseed oil, four parts of tung oil, seven parts of soja bean oil and from eighteen to twenty-four parts 105 of the thinning vehicle to one hundred parts of the pigment.

Highly satisfactory results have been at- 110 tained by me in using a lead pigment, lin- seed oil, tung oil, soja bean oil and a thin- ning vehicle substantially in the proportion, by weight, of about nine parts of linseed oil, eight parts of tung oil, sixteen parts of soja bean oil and twenty-four parts of the thin- ning vehicle to one hundred parts of the 115 lead pigment.

The best results have been attained by me in mixing the linseed oil and the pigment and then thinning the mixture of pigment and linseed oil by adding about one-half of 110

the thinning vehicle to be used in making my improved paint and thereby placing said mixture in the best possible condition for the addition of the tung oil, soja bean oil and 5 the remainder of the thinning vehicle to be used. Thereupon, to attain the best results, the tung oil and the soja bean oil are mixed independently of the thinned mixture of linseed oil and pigment, and then the oil-mix- 10 ture of tung oil and soja bean oil is added and mixed with the thinned mixture of pigment and linseed oil preparatory to adding the remainder of the thinning vehicle.

The most approved embodiment of my in- 15 vention therefore consists in a suitably thinned paint which comprises a thinned mixture comprising a lead pigment and linseed oil and also comprises an oil-mixture comprising tung oil and soja bean oil, with 20 the oils of said mixtures and the pigment substantially in the proportion, by weight, of eight parts of the tung oil, sixteen parts of the soja bean oil and nine parts of the linseed oil to one hundred parts of the pig- 25 ment.

I would here remark, however, that I have attained good results from a paint made by me and comprising a mixture comprising a lead or zinc pigment and linseed oil, an oil- 30 mixture comprising tung oil and paraffin oil, and a thinning vehicle, with the thinning vehicle, the pigment and the linseed oil substantially in the proportion, by weight, of from nine to twelve parts of linseed oil and 35 from eighteen to twenty-four parts of the thinning vehicle to one hundred parts of the pigment, with the quantity of tung oil used equal, by weight, to more than three per cent. of the amount of pigment used, and 40 with the quantity of paraffin oil used not less, by weight, than the quantity of tung oil used.

What I claim is:—

1. A paint comprising a metallic pigment, 45 tung oil, an oil adapted to retard the drying of the tung oil, a drying oil other than tung oil, substantially in the proportion, by weight, or from four to fourteen parts of the tung oil, from seven to thirty-five 50 parts of the oil adapted to retard drying of

the tung oil, and from nine to twelve parts of the second-mentioned drying oil, to one hundred parts of the pigment.

2. A paint comprising a metallic pigment, tung oil, soja bean oil, and a drying oil other 55 than tung oil, substantially in the proportion, by weight, of from four to fourteen parts of the tung oil, from seven to thirty-five parts of the soja bean oil and from nine to twelve parts of the second-mentioned 60 drying oil, to one hundred parts of the pigment.

3. A paint comprising a metallic pigment, tung oil, an oil adapted to retard drying of 65 the tung oil, and a drying oil other than tung oil, substantially in the proportion, by weight, of about eight parts of the tung oil, about sixteen parts of the oil adapted to retard drying of the tung oil, and about nine parts of the second-mentioned drying 70 oil, to one hundred parts of the pigment.

4. A paint comprising a metallic pigment, tung oil, soja bean oil, and a drying oil other than tung oil, in the proportion, by weight, of about nine parts of the last-mentioned oil, 75 about sixteen parts of the soja bean oil and about eight parts of the tung oil, to one hundred parts of the pigment.

5. A paint comprising a metallic pigment, tung oil and an oil adapted to retard 80 drying of the tung oil and a drying oil other than tung oil, with the second-mentioned drying oil and the pigment substantially in the proportion, by weight, of from nine to twelve parts of said second-mentioned 85 drying oil to one hundred parts of the pigment, with the quantity of tung oil used equal, by weight, to more than three and not over about fourteen per cent. of the amount of pigment used, and with the quantity of 90 oil used to retard drying of the tung oil not less, by weight, than the quantity of tung oil used.

In testimony whereof, I sign the foregoing specification, in the presence of two witnesses. 95

WALTER E. WRIGHT.

Witnesses:

CASPER J. DOVER,  
B. C. BROWN.